



US005223055A

# United States Patent [19]

Charquet et al.

[11] Patent Number: 5,223,055

[45] Date of Patent: Jun. 29, 1993

[54] **METHOD OF MAKING A SHEET OR STRIP OF ZIRCALOY WITH GOOD FORMABILITY AND THE STRIPS OBTAINED**

[75] Inventors: Daniel Charquet, Albertville; Marc Perez, Levallois, both of France

[73] Assignee: Compagnie Europeenne du Zirconium Cezus, Courbevoie, France

[21] Appl. No.: 730,595

[22] Filed: Jul. 16, 1991

[30] Foreign Application Priority Data

Jul. 17, 1990 [FR] France ..... 90 09353

[51] Int. Cl.<sup>5</sup> ..... C22C 16/00

[52] U.S. Cl. ..... 148/672; 148/421; 420/422

[58] Field of Search ..... 148/11.5 F, 12.7 B, 148/133, 672, 421; 420/422

[56] References Cited

U.S. PATENT DOCUMENTS

4,584,030 4/1986 McDonald et al. ..... 148/11.5 F  
4,649,023 3/1987 Sabol et al. ..... 420/422  
4,717,428 1/1988 Comstock et al. ..... 148/11.5 F  
4,775,428 10/1988 Bunel et al. ..... 148/11.5 F

4,881,992 11/1989 Bunel et al. ..... 420/421  
4,981,527 1/1991 Charquet ..... 148/11.5 F  
5,080,861 1/1992 Garde ..... 420/422

FOREIGN PATENT DOCUMENTS

0085553 8/1983 European Pat. Off. .

2575764 7/1986 France .

2578555 9/1986 France .

Primary Examiner—Upendra Roy

Attorney, Agent, or Firm—Dennison, Meserole, Pollack & Scheiner

[57] ABSTRACT

A method of making a strip of ZIRCALOY 2 or 4 is disclosed wherein an ingot is worked, roughly shaped into a billet then quenched from the beta range, hot rolled in alpha range, annealed and cold rolled to 0.3 to 0.9 mm. The O and C, in ppm, are selected to satisfy the formula:  $O_2 < 1200 - 0.75 \times C (R)$  so that a T texture is obtained systematically for thicknesses of at least 0.8 mm. The disclosure also concerns the strips obtained. The method can be applied to obtaining strips of excellent formability for the production of components for nuclear water reactors.

17 Claims, 2 Drawing Sheets



x T texture  
+ L tendency  
● L texture

FIG. I



FIG. 2



FIG. 3



**METHOD OF MAKING A SHEET OR STRIP OF ZIRCALOY WITH GOOD FORMABILITY AND THE STRIPS OBTAINED**

**BACKGROUND OF THE INVENTION**

The subject of the invention is a method of making a strip of zircaloy 2 or 4 with good formability.

In the publication by CHARQUET D., AL-  
HERITIERE, E., and BLANC, TG., "Cold-Rolled  
and Annealed Textures of Zircaloy-4 Thin Strips",  
Zirconium in the Nuclear Industry: Seventh Interna-  
tional Symposium ASTM STP 936 R.B., Adamson and  
L.F.P. Van Swan, Eds., American Society for Testing  
of Materials, Philadelphia, 1987, pages 663-672, the  
authors state that the texture of zircaloy strips has a  
great effect on their mechanical properties and form-  
ability.

The T texture of crystal orientation is similar to that  
of pure zirconium; in it the base poles (0002) are typi-  
cally disoriented by 20° to 40° towards the transverse  
direction, while the [1120] is parallel to the rolling di-  
rection. The T texture has a better breaking load, creep  
strength and deformability (bending or stretch forming)  
than so-called C textures (centred isotropic) or L tex-  
tures (base poles swung towards the rolling direction).  
The effect of cold rolling and annealing on texture is  
also discussed in this document; a return to a T structure  
is no longer possible once an L or C structure has been  
obtained.

An initial T structure is obtained by hot rolling in the  
alpha range, but the preservation of a T structure  
through cold rolling and annealing cycles is uncertain.

Applicants have sought to define the conditions  
which will ensure that the T structure is preserved, so  
that the formability of the corresponding strips of ZIR-  
CALOY 4 or ZIRCALOY 2 can be improved system-  
atically.

It will be recalled that the composition of these two  
alloys is given in the ASTM B 352-79 specifications;  
ZIRCALOY 4 and ZIRCALOY 2 correspond respec-  
tively to grades R 60804 and R 60802.

**SUMMARY OF THE INVENTION**

The subject of the invention is a method of making a  
strip of ZIRCALOY 2 or 4 with good formability in  
which—in a manner known from the above-mentioned  
publication—an ingot is produced and hot worked into  
a billet, typically by forging; the billet is heated to beta  
and water quenched, then hot rolled in the alpha range  
and annealed in the alpha range. It is then cold rolled  
with intermediate annealing operations, to a selected  
thickness from 0.3 to 0.9 mm. According to the inven-  
tion, production of the ingot is carried out such that the  
carbon (C) and oxygen (O<sub>2</sub>) content obtained thereby  
satisfy the formula:

(R) O<sub>2</sub> < 1200 - 0.75xC and preferably (R') O<sub>2</sub> 21  
1150 - 0.75xC, the O and C content being expressed in  
ppm. The strips thus obtained have T textures systemat-  
ically in the case of thicknesses of 0.8 mm and over. In  
cases where the final thickness has to be smaller, the  
three recommended preferred measures should be ap-  
plied, singly or combined generally:

(a) hot rolling the billet at the top of the alpha range  
with rolling starting at a temperature of from 730° to  
795° C.;

moderating the annealing operations to keep the texture  
obtained by the following means:

- (b) carrying out the annealing operation which fol-  
lows hot rolling at a temperature below 640° C.;
- (c) carrying out each intermediate annealing opera-  
tion between cold rolling either at from 600° to  
640° C. for 3 and 4 hours, or at from 650° to 700°  
C., for 1 to 5 minutes, or with any other (tempera-  
ture, time) pair which gives an annealing result  
(hardness, recrystallisation) equivalent to either  
intermediate annealing operation.

To obtain a strip 0.6 mm thick, it is preferable to carry  
out three cold rolling/annealing cycles; thus there  
are two intermediate annealing operations. For a  
thickness of 0.4 mm, 3 or 4 cold rolling/annealing  
cycles are carried out, so there are 2 or 3 interme-  
diate annealing operations.

The solution to formula (R) surprisingly enables a T  
texture to be obtained in a strip at least 0.8 mm thick,  
and this is obtained whether the strip is work hardened  
or in an annealed state. It also enables the T texture to  
be preserved with smaller thicknesses, if the clearly defined  
methods (a), (b), and (c) are followed. In the case of ZIRCALOY 4, maintenance of the T texture goes  
together with the presence and maintenance of precipi-  
tates based on (Fe, Cr), which also give an improve-  
ment in the resistance to uniform corrosion in water of  
PWR reactors.

The range defined by (R) is normally limited by the  
maximum C content defined by ASTMB specification  
352, namely 270 ppm. Obtaining the minimum mechani-  
cal properties required for some types of strip for the  
production of grids holding nuclear fuel elements (see  
U.S. Pat. No. 4,717,427 and EP 246986 = U.S. Pat. No.  
4,881,992: E<sub>0,2</sub> at 315° C.  $\geq$  250 MPa, breaking load 315°  
C.  $\geq$  280 MPa), and the wish to avoid Zr carbide precipi-  
tation leads (sic) to the following complementary pre-  
ferred limitations:

40 C  $\leq$  180 ppm and O<sub>2</sub>  $\geq$  600 ppm,

which respectively enhance ductility and increase me-  
chanical strength at 315° C., taking into account the  
texture produced by formula (R). If the best possible  
formability is to be obtained, it is advisable for the selec-  
tion of (C) and (O<sub>2</sub>) content according to the invention  
to be combined with the cold rolling conditions already  
described by Applicants:

either, in accordance with FR 2 575 764, carrying out  
50 the last rolling process with deformation of from 30  
to 55% and the final annealing operation at from 490°  
to 580° C. for 1 to 10 minutes, thereby obtaining  
incipient recrystallisation, which typically involves  
0.5 to 5% of the volume of the strip;

55 or, in accordance with EP 246986 = U.S. Pat. Nos.  
4,775,428 and 4,881,992 (mentioned above), and as an  
alternative form of method (c), with cold rolling  
processes and intermediate annealing operations ad-  
justed so as to have intermediate states where the  
alloy is just recrystallised with very fine grains: carry-  
ing out cold rolling with at least two intermediate  
annealing operations and a final annealing operation,  
each of the two intermediate ones being from 0.5 to  
10 minutes at from 650° to 750° C., the amount of  
deformation between annealing operations being  
from 20 to 55% before the penultimate one, from 30  
to 55% between the last two intermediate ones and  
between the last intermediate one and the final one,

the final annealing operation being from 1.5 to 7 minutes at from 590° to 630° C. and producing partial recrystallisation of the strip obtained, involving 20 to 40% of its volume.

In these cold rolling methods each amount of deformation is calculated by the formula:

$(1 - e/E) \times 100$  where  $e$  and  $E$  are respectively the thicknesses after and before rolling.

It will be seen from the tests that, when the O content (ppm) is increased above (1150 - 0.75xC), L textures are obtained, or T textures which are easily degraded by cold rolling. When the O content is only increased thus by less than 200 to 250 ppm relative to (1150 - 0.75xC), the T texture can still be obtained provided that the transformation conditions are selected, whereas beyond that increase only L texture is possible.

It should be noted, of the products obtained according to the invention, two grades of strip are particularly important:

A. Annealed strips of ZIRCALOY 2 or 4 from 0.3 to 0.9 mm thick, which satisfy the mechanical properties at 288° C. (550° F.) laid down by ASTM specification 352:

|                                                 |         |
|-------------------------------------------------|---------|
| breaking load in longitudinal direction (L)     | 186 MPa |
| breaking load in transverse direction (T)       | 179 MPa |
| and elastic limit at 0.2% (YS) in direction (L) | 103 MPa |
| and elastic limit at 0.2% (YS) in direction (T) | 120 MPa |

having a T texture with  $O_2 \geq 700$  ppm and  $O_2 < 1150 - 0.75xC$ ;

B. Strips of annealed ZIRCALOY 2 or 4 with incomplete recrystallisation or "restored" strips, again from 0.3 to 0.9 mm thick, satisfying the following minimum mechanical properties:

$E_{0.2}$  at 315° C.: 250 MPa, breaking load R in direction (L) 310 MPa, and also having a T texture with  $O_2 \geq 700$  ppm and  $O_2 < 1150 - 0.75xC$ .

The amount of recrystallisation is then 0.5 to 40% of the volume.

The essential advantage of the invention is that it systematically gives strips of ZIRCALOY 4 or ZIRCALOY 2 with the required level of mechanical properties and excellent formability. Formability can typically be assessed by testing their suitability for drawing operations, for example by the ERICHSEN tests. The improvement in formability is accompanied by an improvement in resistance to uniform corrosion.

#### BRIEF DESCRIPTION OF THE DRAWINGS

FIG. 1 is a graph showing the compositions of sheets or strips of Table 1;

FIG. 2 is a diagram of a T texture;

FIG. 3 is a diagram of an L texture.

#### DESCRIPTION OF THE PREFERRED EMBODIMENTS

The following examples concern sheets or strips of ZIRCALOY 4, obtained from a plurality of casting operations, the numbers of which are given in Table 1.

The graph in FIG. 1 shows the content pairs (C,O) of the various sheets or strips in Table 1, with the straight lines forming the limits of formulas (R) and (R') shown respectively as R and R'.

FIG. 2 represents a T texture and FIG. 3 an L texture; these two diagrams are taken from the publication quoted at the beginning of this specification.

The texture in FIG. 2, described as a "T texture", has two base poles (0002) 1 and 2 which are disoriented by 20° to 40° in the transverse direction TD. There are two curves of relative maxima 3 and 4.

The so-called "L texture" in FIG. 3 is very different: the two base poles 5 and 6 are disoriented by 10° to 20° in the rolling direction LD, while the relative maxima 7 and 8 surround the poles 5 and 6 and are closer to them.

In all cases the ingot is roughly shaped hot into a billet, the billet is quenched from beta range then hot rolled in the alpha range to a thickness of 0.4 to 6 mm, and the rolled ingot or rough rolled strip is annealed at 630° C.

As indicated in the above-mentioned publication, recrystallisation of a cold rolled material with a T texture does not markedly change the orientation of the base poles (002). Conversely, when an L texture or a centred texture has been obtained it is not possible to return to a T texture, for example through annealing.

Samples 1 to 6 and 8 in Table 1, which have an O and C content complying with formula (R) and with preferred formula (R'), have a T texture at a thickness of 0.8 mm, either in the annealed state (Samples 1 to 5 and 8) or in the work hardened state (Sample 6): as indicated above, the T texture is that of all the samples both in the work hardened and annealed state.

Sample 7 (0.4 mm thick) illustrates the fact that with further cold rolling the texture may change to an L texture. The change is very evident in this case.

In the case of Sample 10, which is examined at a thickness of 2 mm in the annealed state and a thickness of 1.2 mm in the work hardened state, the change in texture with rolling is premature in view of the strip thicknesses used for spacing grids of nuclear fuel elements (0.3 to 0.9 mm thick).

Samples 9 and 11 to 15 show that, in the case of thicknesses from 0.4 mm to 1.5 mm, an L texture is observed, the corresponding (C,N) pairs being located above the limit line R (FIG. 2).

#### APPLICATIONS

The invention makes it possible to obtain sheets and strips of ZIRCALOY 4 or ZIRCALOY 2 with excellent formability, for producing components for use in nuclear water reactors of the PWR or BWR type, for example spacing grids or casings.

TABLE 1

| SAMPLE REF. | CASTING NO. | O (ppm) | C (ppm) | TYPE OF TEXTURE | THICKNESS (mm) | STATE AND METHOD OF OBTAINING IT |
|-------------|-------------|---------|---------|-----------------|----------------|----------------------------------|
| 1           | 30          | 790     | 57      | T               | 0.8            | Annealed (2 mm)                  |
| 2           | 48          | 930     | 49      | T               | 0.8            | "                                |
| 3           | 978         | 1000    | 155     | T               | 0.8            | "                                |
| 4           | 85          | 1025    | 102     | T               | 0.8            | "                                |
| 5           | 82          | 1060    | 80      | T               | 0.8            | "                                |
| 6           | 33          | 1090    | 35      | T               | 0.8            | Work hardened (2 mm)             |

TABLE 1-continued

| SAMPLE REF. | CASTING NO. | O (ppm) | C (ppm) | TYPE OF TEXTURE | THICKNESS (mm) | STATE AND METHOD OF OBTAINING IT              |
|-------------|-------------|---------|---------|-----------------|----------------|-----------------------------------------------|
| 7           | "           | "       | "       | ?               | 0.4            | "                                             |
| 8           | 58          | 1095    | 60      | T               | 0.8            | Annealed (2 mm)                               |
| 9           | 86          | 1210    | 101     | L               | 0.6            | Partially annealed (0.5 to 5% recrystallised) |
| 10          | 87          | 1320    | 150     | T/L             | 2/1.2          | Annealed/work hardened                        |
| 11          | 79          | 1285    | 90      | L               | 1.0            | Work hardened (2 mm)                          |
| 12          | 25          | 1300    | 120     | "               | 0.8            | Partially annealed                            |
| 12 bis      | "           | "       | "       | L               | "              | Work hardened (2 mm)                          |
| 13          | 10          | 1350    | 96      | L               | 1.5            | Work hardened (2 mm)                          |
| 14          | 17          | 1430    | 114     | L               | 1.2            | Work hardened (2 mm)                          |
| 15          | 678         | 1490    | 77      | L               | 0.4            | Work hardened (2 mm)                          |

## What is claimed is:

1. A method of making a strip of zircaloy 2 or 4 with good formability, comprising the steps of producing an ingot, hot working the ingot to form a billet, quenching the billet from beta range, hot rolling the quenched billet in alpha range, then annealing and cold rolling with intermediate annealing operations to form a strip having a thickness from 0.3 to 0.9 mm;

wherein the production of the ingot is carried out such that:

$$O_2 < (1200 - 0.75C),$$

O<sub>2</sub> and C being expressed in ppm.

2. The method of claim 1 wherein

$$O_2 < 1150 - 0.75xC$$

3. The method of claim 1 or 2, wherein C ≤ 270 ppm.

4. The method of claim 1 or 2, wherein the billet is hot rolled to a thickness from 3 to 6 mm at the top of the alpha range, the temperature at which rolling is commenced being from 730° to 795° C.

5. The method of claim 3, wherein the billet is hot rolled to a thickness from 3 to 6 mm at the top of the alpha range, the temperature at which rolling is commenced being from 730° to 795° C.

6. The method of claim 4, wherein cold rolling is carried out with at least one intermediate annealing operation, each intermediate annealing operation being at from 600° to 640° C. for 3 to 4 hours.

7. The method of claim 4, wherein the last cold rolling step is carried out with deformation of 30 to 55%, and wherein the rolled strip is then subjected to a final heat treatment for 1 to 10 minutes at from 490° to 580° C., thus giving a strip which is partially recrystallized over 0.5 to 5% of its volume.

8. The method of claim 4, wherein cold rolling is carried out with at least two intermediate annealing operations and a final annealing operation, each of the two intermediate ones being for 0.5 to 10 minutes at from 650° to 750° C., the amount of deformation between these operations being from 20 to 55% before the penultimate intermediate annealing operation, from 30 to 55% between the last two intermediate ones and between the last intermediate one and the final one, the final annealing operation being for 1.5 to 7 minutes at from 590° to 630° C. and then producing partial recrystallization of the strip obtained, involving 20 to 40% of its volume.

9. The method of claim 4, wherein cold rolling is carried out with at least one intermediate annealing operation, each intermediate annealing operation being at from 650° to 700° C. for 1 to 5 minutes.

10. The method of claim 4, wherein the annealing operation which follows hot rolling is carried out at a temperature below 640° C.

11. The method of claim 10 wherein the thickness at the end of cold rolling is less than 0.8 mm, and wherein cold rolling is effected with at least two intermediate annealing operations, each intermediate annealing operation being at from 600° to 640° C. for 3 to 4 hours.

12. The method of claim 10, wherein cold rolling is carried out with at least one intermediate annealing operation, each intermediate annealing operation being at from 600° to 640° C. for 3 to 4 hours.

13. The method of claim 10 wherein the thickness at the end of cold rolling is less than 0.8 mm, and wherein cold rolling is effected with at least two intermediate annealing operations, each intermediate annealing operation being at from 650° to 700° C. for 1 to 5 minutes.

14. The method of claim 10, wherein the last cold rolling step is carried out with deformation of 30 to 55%, and wherein the rolled strip is then subjected to a final heat treatment for 1 to 10 minutes at from 490° to 580° C., thus giving a strip which is partially recrystallized over 0.5 to 5% of its volume.

15. The method of claim 10, wherein cold rolling is carried out with at least two intermediate annealing operations and a final annealing operation, each of the two intermediate ones being for 0.5 to 10 minutes at from 650° to 750° C., the amount of deformation between these operations being from 20 to 55% before the penultimate intermediate annealing operations, from 30 to 55% between the last two intermediate ones and between the last intermediate one and the final one, the final annealing operation being for 1.5 to 7 minutes at from 590° to 630° C. and then producing partial recrystallization of the strip obtained, involving 20 to 40% of its volume.

16. A method of making a strip of zircaloy 2 or 4 with good formability, comprising the steps of producing an ingot, hot working the ingot to form a billet, quenching the billet from beta range, hot rolling the quenched billet in alpha range, then annealing and cold rolling with intermediate annealing operations to form a strip having a thickness from 0.3 to 0.9 mm;

wherein the production of the ingot is carried out such that:

$$O_2 < (1200 - 0.75C),$$

O<sub>2</sub> and C being expressed in ppm, and wherein O<sub>2</sub> ≤ 660 ppm and C ≤ 180 ppm.

17. The method of claim 16, wherein the billet is hot rolled to a thickness from 3 to 6 mm at the top of the alpha range, the temperature at which rolling is commenced being from 730° to 795° C.

\* \* \* \* \*